# EUROPEAN PATENT SPECIFICATION

(11) **EP 0 033 040 B1**
(45) Date of publication and mention of the grant of the patent: **22.05.1985**
(21) Application number: 80304782.8
(22) Date of filing: 31.12.1980
(51) Int. Cl.: C23C 2/22

(54) **Improvements in and relating to the wiping of treated wire or strip**
Abstreifen behandelter Drähte oder Bänder
Essuyage de fils ou bandes traités

(30) Priority: 22.01.1980 NZ 192670; 09.09.1980 NZ 194893
(43) Date of publication of application: 05.08.1981
(73) Proprietor: New Zealand Wire Industries Limited, Auckland (NZ)
(72) Inventor: Peel, Colin Dudley, Auckland (NZ); Gin, Colin, Auckland (NZ)
(74) Representative: Brown, John David

## Description

This invention relates to the wiping of a metal coating applied to wire or strip.

The invention has particular although not exclusive application to the wiping of coated wire or strip, as it emerges from a bath of molten metal, such as for example zinc or some other suitable metal coating material.

Up until this time, in the galvanising of wire or coating of wire, the wire or strip has been taken from the bath at a relatively shallow angle to the horizontal and wiped with an asbestos pad or asbestos string.

In the case of asbestos string for example, the asbestos string is wound around the wire and the wire passed through a slot between a pair of fingers, so that the string is wedged into the slot, this wiping the surface of the wire or strip. In the case of pads, these have generally been formed by hand, by winding asbestos card into a pad or disc, the pad or disc then being placed in an suitable pad holder.

European patent specification No. 0,009,940 discloses a method of making a material in the form of refractory fibrous material, including alumino silicate fibrous materials.

It is an object of this invention to go someway towards providing a method for the wiping of coated wire or strip as it emerges from a bath of molten metal and to provide a method for forming a material for use in such wiping of coated wire or strip.

It is a further object of the invention to provide the public and manufacturers with a useful choice.

Other objects of this invention will become apparent from the following description.

According to one aspect of this invention there is provided a method of wiping coated wire or strip, emerging from a bath of molten metal, using a pad including compressed alumino silicate fibres.

According to a further aspect of this invention, there is provided a method of forming a pad for the wiping of coated wire or strip as it emerges from a bath of molten metal, including the steps of:
(a) feeding an amount of material including fibrous alumino silicate, and
(b) compressing said material under pressure to form an integral pad.

The invention will now be described by way of example only, and it should be appreciated that modifications or improvements may be made to the invention without departing from the scope thereof, as defined by the appended claims.

It has been found in experimentation, that compressed, non-combustible material, consisting essentially of alumino silicate fibrous material, has particular advantages in the wiping of wire or strip, which has been coated with a suitable coating, such as zinc or some other metal coating, as it emerges from a bath of molten metal, such as during the processing of wire or strip.

In one form of the invention, the compression of the material including the alumino silicate fibrous material is carried out by a press which consists of a piston moving within a tubular member or housing of a cross section corresponding substantially to that of the resulting pad.

The pressure applied to the material will vary depending upon the size of the material and also upon the size of the wire to be wiped.

The compression and thus compacting of the material causes a resultant pad or disc to remain as an integral unit during wiping of coated wire or strip.

For large diameter wires, the pads are preferably softer (that is to say compressed at a lower pressure), than would be the case for pads suitable for small diameter wires.

The pad is thus formed of a non-combustible material, consisting essentially of an alumino silicate fibrous material.

The alumino silicate fibrous material is fed to a compression station or means, and then compressed by applied pressure into a pad or disc. If desired a suitable lubricant, such as powdered graphite can be added to the alumino silicate fibrous material.

The present method provides for the use of such a compressed pad consisting essentially of alumino silicate fibrous material in the wiping of coated wire or strip, such as it emerges from a bath of molten metal. For example, as in the galvanising of wire or strip. The method of wiping coated wire or strip according to the present invention has a number of advantages. By way of example, the advantages are:
1. The use of alumino silicate fibrous material removes or at least reduces substantially health hazards which are present by using asbestos material such as used up until this time.
2. It has been found during experimentation that use of alumino silicate fibrous material, as a pad wiping material, enables the pad wiping material to withstand temperatures generally higher than asbestos or other material. For example, it has been found that alumino silicate fibrous material can generally withstand high temperatures (such as found during wiping operations) of up to approximately 1300°C.
3. The use of alumino silicate fibrous material as a pad wiping material has generally been found to give a longer and higher pad life than other pad wiping materials (such as asbestos).
4. By using alumino silicate fibrous material as a pad wiping material, it has been found that a more even wipe is obtained over the wire or strip, than is generally obtained by using other materials (such as asbestos).
5. The use of alumino silicate fibrous material results in a tighter wipe about the wire or strip, and generally speaking results in a low coating thickness as compared with other materials.

Preferably, in use alumino silicate fibre material, the material is compressed into a pad or disc by an applied pressure in the range of about 7 to 20 tonnes per square inch (1x10⁸ to 3x10⁸ Nm-²). This is however by way of example only.

It will be appreciated that the compacting of the alumino silicate fibrous material causes the pad to remain as an integral unit during wiping.

In use, it has been found to be advantageous to add a lubricant, such as for example powdered graphite. This is advantageous for example at the beginning of a wiping operation, when the wire or strip begins to pass through or past the pad.

## Claims

1. A method of wiping coated wire or strip, emerging from a bath of molten metal, using a pad including compressed alumino silicate fibres.

2. A method as claimed in claim 1, wherein said pad further includes a lubricant.

3. A method as claimed in claim 2, wherein the lubricant is powdered graphite.

4. A method of forming a pad for the wiping of coated wire or strip as it emerges from a bath of molten metal, characterised in that said method includes the steps of:
(a) feeding an amount of material including alumino silicate fibrous material, and
(b) compressing said material under pressure to form an integral pad.

5. A method as claimed in claim 4, wherein said pressure is in the range of 7 to 20 tonnes per square inch (1x10⁸ to 3x10⁸ Nm-²).

## Revendications

1. Méthode d'essuyage d'un fil ou ruban métallique enrobé émergeant d'un bain de métal fondu, utilisant un tampon contenant des fibres d'aluminosilicate compressées.

2. Méthode selon la revendication 1, dans laquelle ledit tampon comprend en outre un lubrifiant.

3. Méthode selon la revendication 2, dans laquelle ledit lubrifiant est du graphite pulvérisé.

4. Méthode de fabrication d'un tampon pour l'essuyage d'un fil ou ruban métallique lorsqu'il émerge d'un bain de métal fondu, caracterise par le fait que ladite méthode comprends les étapes de:
(a) introduction d'une quantité de matériau comprenant un matériau fibreux d'aluminosilicate et
(b) compression dudit matériau sous pression pour former un tampon d'une seule pièce.

5. Méthode selon la revendication 4, dans laquelle ladite pression varie de 7 à 20 tonnes au pouce carré (1×10⁸ à 3×10⁸ Nm⁻²).

## Patentansprüche

1. Ein Abstreifverfahren für überzogene Drähte oder Bänder, die aus einem Bad geschmolzenen Metalls austreten, welches einen komprimierte Aluminiumsilikatfasern aufweisenden Stoff verwendet.

2. Ein Verfahren wie in Anspruch 1 beansprucht, wobei dieser Stoff ferner ein Schmiermittel umfaßt.

3. Ein Verfahren wie in Anspruch 2 beansprucht, wobei das Schmiermittel gepulvertes Graphit ist.

4. Ein Verfahren zur Herstellung eines Stoffes zum Abstreifen überzogener Drähte oder Streifen, wenn sie aus einem Bad geschmolzenen Metalles austreten, dadurch gekennzeichnet, daß das Verfahren die Schritte:
(a) Zuführen einer Materialmenge, welche faserartiges Aluminiumssilikatmaterial einschließt, und
(b) Komprimieren des Materials unter Druck, um ein einstückiges Stoffstück herzustellen, aufweist.

5. Ein Verfahren wie in Anspruch 4 beansprucht, wobei der Druck im Bereich von 7 bis 20 Tonnen pro Quadrat-Inch (1×10⁸ bis 3x10⁸ Nm-²) liegt.
